

# UNITED STATES PATENT OFFICE

CLYDE J. COLEMAN, OF NEW ROCHELLE, NEW YORK, ASSIGNOR TO STERN-COLEMAN  
DIAMOND MACHINE COMPANY, INC., OF NEW YORK, N. Y.

## ART OF POLISHING DIAMONDS.

1,329,373.

Specification of Letters Patent.

Patented Feb. 3, 1920.

No Drawing.

Application filed June 15, 1915. Serial No. 34,161.

To all whom it may concern:

Be it known that I, CLYDE J. COLEMAN, a citizen of the United States, and a resident of Premium Point Park, New Rochelle, 5 Westchester county, New York, have invented certain new and useful Improvements in the Art of Polishing Diamonds, of which the following is a specification.

In polishing diamonds, it is the practice at the present time to hold the diamond in the polishing tool by partially embedding it in a body of metal in a semi-molten state, contained in a small brass basin or dop, the diamond being held in position by the metal after the metal has cooled. This method suffers from the disadvantage that it is necessary from time to time to soften the metal and readjust the diamond, to expose a different part thereof for polishing, as it is not possible to expose at one time all parts of the diamond on one side of the girdle line. It is also common practice to lock the larger stones in a clamping device, but this device is very difficult to adjust so as to hold the diamond at the correct angle. The difficulty in holding diamonds during the polishing operation, as distinguished from other precious stones, is due to the extreme hardness of the diamond which necessitates applying great pressure, with resultant great friction and generation of great heat. Diamond polishing is particularly a difficult operation and unlike any other lapidary work because with all other gems there is something harder than they are, which will easily abrade them and not require any special speed or pressure to polish them, but the diamond being the hardest known substance, it must be polished with its own dust. This requires great lap speed, great pressure and also a precise grain presentation to the direction of movement of the lap, with the result that a high temperature is generated and often an almost instantaneous rise from low red heat to white red heat is developed when a hard spot is encountered and then dropping back suddenly to the normal red heat. Therefore a cement must possess resistance against the disintegrating effect of great vibration, must be refractory enough to resist the heat of polishing, must be strong and adhesive to resist the pressure and strain and must have substantially the same coefficient of expansion or a requisite degree of elasticity which is equivalent thereof, so that its

adhesion will not be destroyed or impaired by expansion or contraction due to such temperature changes.

The object of the invention is to provide an improved method for holding diamonds in position for polishing, so as to avoid the disadvantages of the prior methods, and in particular to make it possible to polish all faces of the diamond on one side of the girdle line without reclamping or resetting the diamond in its holder, thereby avoiding the troublesome adjustments, calling for skilled manipulation, heretofore necessary.

To these ends the invention contemplates attaching the diamond to the arbor by means of the adhesive action of a cement having the physical characteristics that it does not disintegrate or soften under the heat of the polishing operation, and has a coefficient of expansion so near that of the diamond or such a degree of elasticity that the diamond during the polishing may be rigidly held in place by the cement applied to the diamond on one side of the girdle, whereby substantially all the facets on one side of the girdle may be polished without resetting or reclamping the diamond to the arbor.

I find that a cement having clay as the principal base gives excellent results in such a method of securing the diamond to the arbor. With the clay base there is preferably employed a binder such as a compound in the nature of an enamel, preferably borax and nitrate of antimony. However, other binders may be used to increase the adhesive properties of the cement. The cement also preferably contains graphite or its equivalent.

One method of compounding such a cement is as follows: take 50 parts by bulk of Dixon's stove polish (composed of 60% clay and 40% graphite), selecting that which is dense, hard and of good body, and not friable, crumbly, sooty or of a dirty nature, and 50 parts by bulk of pure white soapstone clay, such as the talcum and steatite varieties, and 20 parts by bulk of borax or boric acid, and 10 parts by bulk of nitrate of lead, and with these in finely divided condition, mix them thoroughly. Nitrate of antimony is then prepared in the form of a concentrated solution, by allowing strong nitric acid to act on an excess of antimony for about ten to sixteen days, and this solution diluted by adding about an equal amount of water.

The powdered mixture is then made into a thick, creamy paste with a sufficient amount of the nitrate of antimony solution. This paste is allowed to stand for 24 hours or 5 longer, and then it is made again into a similar paste with water.

Good results have been obtained by omitting the nitrate of lead and using the nitrate of antimony alone with the clay, graphite and borax. Thus 32 parts by weight of the 10 Dixon's stove polish, 16 parts by weight of clay, and 12 parts by weight of borax may be mixed with the nitrate of antimony solution as above described. Obviously other 15 materials than those mentioned may be used to mix with the clay to bring out its adhesive qualities, hence the invention is not limited to the precise materials and quantities named.

20 The paste is placed between the diamond and the arbor, preferably being applied in considerable body, so that it will be anchored in the arbor and will form a stem within the arbor for adhesively holding the diamond, and it is baked with the parts held together, at a high temperature, preferably in a non-oxidizing environment, as by enclosure in a retort containing carbon monoxide or nitrogen gas. The heat is first applied at a low temperature to dry the material and is gradually increased to 800° F. or higher. The baking usually requires from 25 to 30 minutes. The cement is preferably gradually cooled.

35 While I have described in detail certain formulas for the cement, which may be used in my improved method of securing the diamonds for polishing, it will be understood that other cements having the characteristics mentioned may well be used, as well as similar cements containing other materials, and cements containing the same materials, but in different quantities. Accordingly, my invention in its broader aspects is not limited to the details described.

45 Having fully and clearly described my invention, what I claim as new and desire to secure by Letters Patent is:

1. The method of securing diamonds for 50 the polishing operation which consists in attaching the diamond to a suitable arbor by means of a cement capable of adhesion to the diamond surface, after baking, with

tenacity sufficient to resist the stress of the polishing of the diamond, and baking the 55 cement to cause the diamond to thus rigidly adhere thereto.

2. The improved method of securing diamonds during the polishing thereof, which consists in securing the diamond to a suitable arbor by means of the adhesive action 60 of a cement, then polishing substantially all the facets on one side of the girdle of the diamond without resetting the diamond, resetting the diamond and securing it by means of the adhesive action of cement, so as to present for polishing the facets on the other side of the girdle and then polishing substantially all the facets on said last mentioned side of the girdle of the diamond 70 without resetting the diamond.

3. The improved method of securing diamonds during the polishing thereof, which consists in securing the diamond to a suitable arbor by means of the adhesive action 75 of a cement baked to the diamond, then polishing substantially all the facets on one side of the girdle of the diamond without resetting the diamond, resetting the diamond and securing it by means of the adhesive action of cement baked to the diamond, so as to present for polishing the facets on the other side of the girdle and then polishing substantially all the facets on said last mentioned side of the girdle of the diamond without resetting the diamond.

4. The method of polishing diamonds which consists in attaching the diamond to the holding means by adhesion wholly on one side of the girdle, polishing the facets 90 on the other side of the girdle, attaching the diamond to the holding means on the polished side of the girdle, and polishing the facets on the other side of the girdle.

5. The method of polishing diamonds 95 which consists in attaching the diamond to the holding means with cement wholly on one side of the girdle, polishing the facets on the other side of the girdle, attaching the diamond to the holding means on the polished side of the girdle, and polishing the facets on the other side of the girdle.

In testimony whereof I have signed my name to this specification.

CLYDE J. COLEMAN